

## UNITED STATES PATENT OFFICE

WYLY M. BILLING, OF CINCINNATI, OHIO, ASSIGNOR TO THE WM. S. MERRELL COMPANY, OF CINCINNATI, OHIO, A CORPORATION OF OHIO

## CASTER-OIL SOAP AND PROCESS OF MAKING CASTOR-OIL SOAP

No Drawing.

Application filed April 14, 1926. Serial No. 102,078.

My invention relates to soaps and the processes for making same. My invention relates particularly to those soaps having germicidal powers or properties wherefore they are used for treatment of various diseases, illnesses and infections.

Certain of these soaps, although soluble in the first instance, if made into a concentrated solution by addition of distilled water, on cooling, develop into a transparent stiff, firm gel, of high viscosity.

One of the objects in making concentrated soap is to have soap in a form that can be conveniently diluted with water to weak solutions.

It is obvious that a gel as indicated will require some time and patience to again take it up in water for forming the weak solution. These weak solutions, while being perfectly fluid, readily attack glass or vitreous surfaces, and in so doing are precipitated, thereby lowering the activity of the solution. Further, the weak solution is hazy, cloudy and turbid.

An object of my invention is to produce a soap that may be given a concentrated fluid or paste form providing a weak solution that will be perfectly clear or transparent and which will not attack glass or vitreous surfaces, with the effects previously noted.

Although I shall explain my discovery and invention as applied to castor oil soap, and in so explaining the invention and the principles involved, the application of my invention to other soaps and analogous or parallel chemical processes readily suggest themselves, wherefore I do not limit myself to the specific or exact substances, proportions, temperatures and steps that I am about to enumerate.

In the application of my invention to castor oil soap it should be borne in mind that at the present time castor oil soap is not commonly found in commerce because no one has shown any advantages in its use. Recently however, a great deal of work has been done to show that castor oil soap has a very definite germicidal power as well as a marked effect in neutralizing bacterial toxins.

It is an object of my invention to so prepare castor oil soap that its stated valuable properties may be utilized. To do this the substance should be in such form that it will readily or freely mix with water, and when so admixed will not attack glass and be thereby precipitated. The significance of this is evident when considering that in hospitals, in clinics, and in ordinary household uses or products of this nature, enamel ware is commonly used for holding solutions. Enamel ware consists of a vitreous or glass surface upon metal.

Castor oil soap is a very water soluble soap, in fact much more so than most other soaps. Potassium soaps are, as a rule, more water soluble than sodium soaps of the corresponding fatty acids, but even castor oil sodium soap is highly soluble. In explaining my invention I shall explain same as it relates to potassium soaps although it is to be understood that the substance of my invention applies likewise to sodium soaps.

Heretofore, in endeavoring to make a concentrated solution of castor oil soap it has been found that castor oil soap, similar to other soaps, when admixed with distilled water in a proportion of about 25% to 40% soap, would give a stiff firm gel; for example, in making a 40% solution, the same on cooling gives a perfectly transparent gel of high viscosity. One of the objects in making a concentrated soap is to have it in a form which would be conveniently diluted to a weak solution. It is obvious that such a gel as is formed by the 40% solution, would require a certain amount of time and patience to again take it up in water and thus form a weak solution. Furthermore, weak solutions, for example 1 to 2%, and in which some of the 40% solution has been utilized, while being perfectly fluid, readily attacks glass, and in so doing the soap is to some extent precipitated. The result is that the activity of the solution is therefore materially lowered.

In practicing my invention, I saponify castor oil by the exact equivalent amount of caustic soda, or potash, for obtaining a true neutral soap. This neutral soap has the dis-

advantages mentioned for ordinary castor oil soaps. To this true neutral soap I add small amounts of free fatty acids derived from the castor oil, as a result of which the 5 gel will undergo a liquefaction. If the small amounts of free fatty acids of the source indicated are added while the solution is hot, the mass will cool off as a liquid. This liquefied gel or solution resulting from the 10 addition of the free fatty acids upon the cooling off of the mass when diluted, provides a solution that remains perfectly clear. Further this diluted solution does not attack 15 glass.

I have found that the following steps and proportions give desirable results.

In making a 40% solution I saponify 80 20 grams of castor oil, with sufficient quantity of sodium hydroxide, which usually amounts to about 10 grams. The sodium hydroxide is dissolved in about 20 cc. of water and added to the castor oil with gentle heat of approximately 100° Fahrenheit. When the oil starts to saponify it goes very rapidly 25 and froths. To prevent it from boiling over I add only a little caustic soda at a time or else keep the mixture barely warm not hot. When tests show that the soda is all used up, I dissolve  $\frac{1}{4}$  to  $\frac{1}{2}$  gram of caustic soda in a few cc. of water and add this a little at a 30 time, until the soap dissolves clear in distilled water, which is very slightly alkaline in alcoholic solution to phenolphthalein.

I then prepare the fatty acids of castor 35 oil by completely saponifying about 80 grams of castor oil with sodium hydroxide 11 grams, the whole of which is dissolved in sufficient quantity to make a dilute soap solution of approximately 5%. I then throw 40 the fatty acids out of solution by adding an excess of sulphuric acid. About 14 grams of the 98% sulphuric acid are required. The fatty acids will rise to the surface and the aqueous solution is drawn off from underneath. The resulting fatty acids are 45 washed by water several times to remove the sulphates and acid. In this way I obtain 75 grams of the fatty acids. I now add about 8 grams of this fatty acid mixture to the 50 soap solution as previously described and allow same to cool. I have found that in this process about 5 grams of fatty acids are used up in neutralizing the slight excess of caustic which I added, thereby leaving 55 about 3 grams additional of fatty acids present. These amounts vary of course with the excesses of caustic which is present. I then add sufficient quantity of water to give about 200 grams of solution containing 40% of 60 castor oil soap. This gives a strong solution of castor oil soap, which mixes readily with water and gives dilutions with great ease, and furthermore, these dilutions do not attack 65 glass as the ordinary castor oil soap does.

I have used potassium hydroxide with equal success but prefer the use of sodium hydroxide because of its substantially more healthy action upon human tissue. I may also produce a 40% solution of sodium ricinoleate by a similar process. Ricinoleic acid occurs in castor oil as a glyceride along with other fatty acids such as stearic, hydroxy stearic, etc. Ricinoleic acid may be purified from these other acids in any suitable manner or by any desired method or process. As such the purified or partly purified acid may be used as a basis of making a 40% solution of sodium ricinoleate of greater purity than is obtainable by direct 80 saponification of castor oil. In this way I have obtained a 40% solution of pure or practically pure sodium ricinoleate, which has all the advantages of fluidity, clarity and non-solvent action on glass, which was 85 explained for the castor oil soap.

What I claim is:

1. As a new article of manufacture a saponified castor oil in a liquid form and comprising approximately 25% to 40% castor 90 oil, approximately 75% to 60% distilled water, sodium hydroxide and free fatty acids of castor oil in excess of the amount necessary to complete reaction of the sodium hydroxide.

2. The process which comprises saponifying 80 grams of castor oil with approximately 10 grams of sodium hydroxide dissolved in water and adding to the castor oil with gentle heat approximately 100° Fahrenheit, and adding small quantities of caustic soda from time to time until the resulting mixture dissolves clear in distilled water, slightly alkaline in alcoholic solution to phenolphthalein and adding thereto 8 105 100 grams of fatty acids and permitting same to cool.

3. As a new article of manufacture, a saponified castor oil in a liquid form and comprising approximately 25% to 40% castor 110 oil, approximately 75% to 60% distilled water, alkaline metal hydroxide and free fatty acids of castor oil in excess of the amount necessary to complete reaction of the alkaline metal hydroxide.

4. As a new article of manufacture, a clear concentrated fluid castor oil soap and being a true neutral soap liquefied by the addition of free fatty acids derived from castor oil and being readily soluble in water 120 to provide a transparent diluted solution.

5. As a new article of manufacture a concentrated castor oil soap solution rendered clear, non-solvent upon glass and freely soluble in water by the presence of an excess of free fatty acid of castor oil.

In testimony whereof, I have hereunto subscribed my name this 10th day of April, 1926.

WYLY M. BILLING.

130